

Patented Nov. 8, 1932

1,886,469

# UNITED STATES PATENT OFFICE

GEORGE R. COULS, OF DETROIT, MICHIGAN

## CUTTING TOOL ALLOY

No Drawing.

Application filed February 27, 1931. Serial No. 518,919.

The invention relates to alloy steels and has for its object the obtaining of an alloy having improved physical characteristics such as fineness of grain, hardness, toughness and rigidity at relatively high temperatures, which characteristics particularly adapt it for use as a cutting tool. My improved product results from the fusing of the following ingredients in substantially the proportions given and in the following manner:

Steel scrap... 26%  
Tungsten... 21% (98% pure)  
Chromium... 31.5% (98% pure)  
Cobalt... 14%  
15 Ferro vanadium... 5% (38% vanadium content)  
Copper... 2.5%

The steel scrap, tungsten, chromium and cobalt are first introduced into the furnace or crucible and heated to a temperature of from 3200° to 3300° F. to fuse and commingle the same. The copper is then added and after an interval of from five to ten minutes the 25 ferro vanadium is introduced. Preferably a small amount of titanium, about 1%, is added to the molten metal before pouring, after which the metal is cast either in bars or suitably fashioned tools.

30 The product resulting from the above process has substantially the proportion of ingredients as introduced, with the exception of a portion of the vanadium and the titanium which are removed with the slag. There is 35 also present a small percentage of carbon. As above stated, the physical characteristics of the alloy are hardness and unusual fineness of its cutting crystals together with toughness in the matrix which permit of 40 forming and maintaining a keen cutting edge on the tool. Furthermore, it maintains its rigidity at fairly high temperatures which adapt it for high speed cutting operations.

45 What I claim as my invention is:

An alloy comprising the following in-

gredients in substantially the following proportions:

|          | Parts         |
|----------|---------------|
| Iron     | 26            |
| Tungsten | 21            |
| Chromium | 31.5          |
| Cobalt   | 14            |
| Vanadium | from 1 to 5   |
| Copper   | from 2 to 2.5 |

In testimony whereof I affix my signature. 55  
GEORGE R. COULS.

60

65

70

75

80

85

90